

[54] SULFUR-HYDROCARBON SLURRY  
PIPELINE TRANSPORTATION  
CONTAINING AN INORGANIC CORROSION  
INHIBITOR

[75] Inventor: Richard J. Horvath, Houston, Tex.

[73] Assignee: Shell Oil Company, Houston, Tex.

[22] Filed: Jan. 8, 1973

[21] Appl. No.: 321,885

**Related U.S. Application Data**

[63] Continuation-in-part of Ser. No. 36,994, May 13, 1970, abandoned.

[52] U.S. Cl. .... 21/2.5 R; 21/2.7 R; 208/47; 208/236; 252/387; 252/8.55 E; 302/14; 302/66

[51] Int. Cl. .... B65g 53/04; C23f 11/16

[58] Field of Search..... 252/387, 8.55 E; 302/14, 302/66; 21/2.5 R, 2.7 R; 208/47, 236

[56] **References Cited**

UNITED STATES PATENTS

2,798,772 7/1957 Redcay ..... 302/14

|           |         |                   |         |
|-----------|---------|-------------------|---------|
| 3,331,657 | 7/1967  | Peter et al. .... | 302/66  |
| 3,438,680 | 4/1969  | Scheverman.....   | 302/66  |
| 3,489,677 | 1/1970  | Thompson .....    | 208/236 |
| 3,539,225 | 11/1970 | Vondrak .....     | 302/66  |
| 3,547,496 | 12/1970 | Kruka .....       | 302/66  |
| 3,547,497 | 12/1970 | Bolger.....       | 302/66  |
| 3,606,482 | 9/1971  | Vondrak .....     | 302/66  |
| 3,606,483 | 9/1971  | Gable et al. .... | 302/66  |

*Primary Examiner*—Benjamin R. Padgett

*Assistant Examiner*—Irwin Gluck

*Attorney, Agent, or Firm*—Fredrik Marlowe

[57]

**ABSTRACT**

A process for preventing plugging and corrosion of conduits used in making and transporting sulfur in the form of a sulfur-liquid hydrocarbon slurry by addition prior to, during, or after preparation of the slurry of a small amount of ammonium polysulfide or ammonium hydrosulfide.

**2 Claims, No Drawings**

**SULFUR-HYDROCARBON SLURRY PIPELINE  
TRANSPORTATION CONTAINING AN  
INORGANIC CORROSION INHIBITOR**

**CROSS-REFERENCE TO RELATED PATENT  
APPLICATION**

This is a continuation-in-part of application Ser. No. 36,994, filed May 13, 1970, and now abandoned.

**BACKGROUND OF THE INVENTION**

The transportation of sulfur neat or as a water or oil slurry in pipelines is well known in the art as noted by reference to U.S. Pat. Nos. 2,798,772; 2,917,345 or 3,947,578, or as described in Pipeline Industry, June, 1967, pages 58-60. In making the sulfur into a sulfur-hydrocarbon slurry, the sulfur is generally sprayed in molten form into either water or a hydrocarbon to form a slurry suitable for transportation through a pipeline. Formation of a stable slurry wherein the sulfur does not undergo any undesirable change, cause corrosion, or does not exhibit a tendency to wide variation in viscosity is essential to the process. In addition other problems may be encountered during preparation and transportation of the slurry through a pipeline. Thus, separation of the sulfur from the carrier fluid, plating or coating of the sulfur on equipment and pipeline walls causing plugging of the pipeline, corrosion, viscosity changes due to pressure and temperature variations encountered requiring increases in pumping power which increases operation costs, etc., are only a few of the problems normally encountered in making sulfur-liquid hydrocarbon slurries for transporting through pipelines.

Although the above are serious problems for consideration in making and transporting sulfur slurries through pipelines, nevertheless, the transportation of sulfur in slurry form through pipelines is an effective, attractive and economic means of transportation, particularly since sulfur is recovered or obtained from isolated, remote and inaccessible areas, and must be transported to desired accessible areas. As noted above, a number of methods have been proposed for making sulfur slurries for pipeline transportation such as injecting molten sulfur into water or a liquid hydrocarbon. Such sulfur slurries when transported through pipelines generally do not overcome the corrosion, coating and/or plugging problems described above.

**OBJECTS OF THE INVENTION**

An object of the present invention is to prepare for pipeline transportation a sulfur-liquid hydrocarbon slurry which is stable, flowable and non-corrosive.

Another object of the present invention is to transport through a pipeline sulfur-liquid hydrocarbon slurries without causing sulfur coating, deposition or plugging or corrosion of the pipeline.

Still another object of the invention is to form a slurry of sulfur in a liquid hydrocarbon medium, which when formed is stable, non-corrosive, does not tend to cause corrosion of preparatory equipment and pipelines and does not cause plugging when the slurry is transported through a pipeline and from which the sulfur can be readily recovered as essentially pure sulfur at the terminal end of the line.

Another object is to transfer sulfur as a liquid hydrocarbon slurry by pipeline over great distances under

non-corrosive conditions and at reduced pumping and handling costs.

Other objects will be apparent from the following description.

5

**SUMMARY OF THE INVENTION**

The present invention is directed essentially to an improved, novel technique for preparing and transporting a sulfur-liquid hydrocarbon slurry through conduits

10 such as pipelines generally over great distances without causing corrosion, coating, deposition or plugging of the slurry equipment, pipeline, etc., due to the tendency of sulfur under such conditions to adhere to equipment and the pipeline walls because of temperature, pressure and other variable conditions so as to corrode and plug said lines by admixing, adding or injecting prior to, during, or after preparation of the sulfur-liquid hydrocarbon slurry or injection into a sulfur-liquid hydrocarbon slurry after it has been injected into 15 a pipeline, a small amount of from about 0.01% to about 10% or higher by weight based on the total slurry, preferably between about 0.1% to about 5% by weight, of an aqueous solution of about 0.1% to about 40% by weight or higher of ammonium hydrosulfide or 20 ammonium polysulfide.

**DESCRIPTION OF THE PREFERRED  
EMBODIMENTS**

It has been found that by injecting or adding about 30 0.1 to 5% by weight based on the total slurry of an ammonium polysulfide solution or ammonium hydrosulfide solution during or after preparation of a sulfur-liquid hydrocarbon slurry or into a pipeline transporting a sulfur-liquid hydrocarbon slurry in which the sulfur content of the slurry can vary from about 10% by weight 35 to about 75% by weight or higher, preferably between about 30 and 70% by weight sulfur, results in inhibition 40 of corrosion and prevention of plugging of the line due to sulfur deposition on the walls of the pipeline and results in improved flowability of the slurry through the pipeline at reduced pumping cost. A highly preferred 45 plugging and corrosion preventing composition of this type is a sulfur-liquid hydrocarbon slurry to which is added from about 0.1 to 2% by weight based on the total slurry of a solution of the above concentration of 50 ammonium polysulfide,  $(NH_4)_xS_y$  wherein  $x$  and  $y$  are integers of at least 2 or more, e.g.  $(NH_4)_2S_y$  wherein  $y$  is 2-8, or ammonium hydrosulfide,  $NH_4HS$ . The corrosion preventing agent is the ammonium polysulfide 55 and not the ammonium hydrosulfide; however, the ammonium hydrosulfide reacts with free sulfur in the slurry to form the polysulfide. The required concentration of ammonium polysulfide, either added or formed in-situ by reaction of free sulfur in the slurry with added 60 ammonium hydrosulfide, to obtain adequate corrosion inhibition and prevent plugging is dependent primarily upon temperature of the slurry, slurry velocity, etc.

The sulfur-liquid hydrocarbon slurry can be made by any suitable means such as described in U.S. Pat. Nos. 2,798,772 or 3,443,827. It is preferred that the method for making the sulfur-liquid hydrocarbon slurry be used in which the sulfur is produced in spherical form since this facilitates the stable dispersion and suspension of the sulfur in the liquid hydrocarbon carrier and inhibits attrition and reduces friction. The phase transfer method for making the sulfur slurry as described in U.S. Pat. No. 3,443,827 provides for first forming a sul-

fur-water slurry and thereafter phase transferring the sulfur particles from the water into a liquid hydrocarbon. In this process the phase transformation to form the sulfur-hydrocarbon slurry can be so controlled that a small amount (1 to 5% by weight basis total slurry) of water is transferred with the sulfur-water phase into the hydrocarbon phase, and thereafter an ammonium hydrosulfide or ammonium polysulfide solution can be added to accomplish the essential desired end of the present invention, namely, corrosion inhibition of sulfur-oil slurries. However, in accordance with the preferred technique of the invention the slurry is formed

1.0% to 45% sulfur was injected. The results of the presence of the ammonium polysulfide solution on corrosion of steel in contact with a sulfur-oil slurry system under varying conditions are shown in Tables 1 and 2.

5 Equally good results are obtained with the above described procedure when ammonium hydrosulfide is substituted for ammonium polysulfide. Good results are also obtained when the addition of corrosion preventing agent is made prior to or during slurry preparation. Under favorable temperature conditions weak solutions of the corrosion preventing agent yield good results.

Table 1

EFFECT OF SULFUR CONTENT OF HIGH STRENGTH AMMONIUM SULFIDE SOLUTIONS ON CORROSION OF CARBON STEEL AT ELEVATED TEMPERATURES

| Temp., °F<br>Solution<br>Comp. %w | Test Conditions                      |       |           |       |           |             |                 |                  |
|-----------------------------------|--------------------------------------|-------|-----------|-------|-----------|-------------|-----------------|------------------|
|                                   | 180                                  |       | 180       |       | 212       |             | 266             |                  |
| NH <sub>3</sub>                   | 14.8                                 |       | 33.3      |       | 33.3      |             | 33.3            |                  |
| H <sub>2</sub> S                  | 12.5                                 |       | 28.1      |       | 28.1      |             | 28.1            |                  |
| Water                             | Remainder                            |       | Remainder |       | Remainder |             | Remainder       |                  |
| Sulfur, <sup>b</sup><br>%w        | Corrosion Rate, mils/yr <sup>a</sup> |       |           |       |           |             |                 |                  |
|                                   | Liquid                               | Vapor | Liquid    | Vapor | Liquid    | Vapor       | Liquid          | Vapor            |
| 0.25                              | 3                                    | —     | 3         | 2     | 4,5,5,7   | 5,41,<br>76 | 6,7,<br>160,270 | 36,56<br>130,130 |
| 0.55                              | 3                                    | —     | —         | —     | —         | —           | 4.9             | —                |
| 0.85                              | 2                                    | —     | 3         | 2     | 4,5,6     | 4,4         | 8,8,8,11,98     | —                |
| 2.85                              | 3                                    | —     | 3         | 2     | 5,5,6     | 4.5         | 6               | 89               |
| 4.85                              | 4                                    | —     | 3         | 2     | 4         | —           | —               | —                |
| 5.85                              | 3                                    | —     | —         | —     | —         | —           | 9,10,10         | —                |
| 6.05                              | 1,2,3                                | 3,3,4 | —         | —     | —         | —           | —               | —                |

<sup>a</sup>From weight loss and exposure time. No localized attack observed.

<sup>b</sup>Sulfur present in solution as polysulfide ion.

by direct spraying of molten sulfur into the hydrocarbon.

The hydrocarbon carrier for the sulfur can be any liquid hydrocarbon ranging from a light petroleum fraction such as liquefied petroleum gas (LPG) to fuel oil, gasoline, kerosene, petroleum distillates, condensates, crude oil and mixtures thereof. Preferred are liquid hydrocarbons containing at least 10% by weight or higher of aromatics, preferably about 15 to 30% by weight aromatic enriched kerosene or crude oil or crude oil condensate fractions containing 15 to 20% by weight aromatics which include mono- and polyaromatic hydrocarbons.

At the terminal end of the line, the aqueous solution can be readily separated from the sulfur-hydrocarbon system by suitable phase separation, distillation or the like.

Slurries of 40 to 60% by weight of sulfur in (a) an aromatic (17% by weight) enriched kerosene or (b) a petroleum condensate or (c) a blend of (b) and crude oil or (d) a crude oil slurry, were prepared by (I) spraying molten sulfur directly into the hydrocarbon, for example crude oil at an oil temperature of about 140°F, to produce sulfur particles, rather spherical in shape, and with an average size of about 50 microns, or (II) by phase transfer by first injecting molten sulfur into an aqueous liquid such as water and thereafter contacting the slurry thus formed with hydrocarbons (a), (b), (c) or (d) to effect phase transfer of the sulfur particles into the hydrocarbon. After preparation of the sulfur-oil slurry, a high strength (25 to 40% NH<sub>3</sub> and 20 to 40% H<sub>2</sub>S) ammonium polysulfide solution containing

40

45

50

55

60

Table 2

EFFECT OF SALT CONTENT OF AMMONIUM POLYSULFIDE SOLUTIONS ON CORROSION OF CARBON STEEL AT ELEVATED TEMPERATURES

| Temperature, °F<br>Solution Composition, %w | Test Conditions                      |           |
|---------------------------------------------|--------------------------------------|-----------|
|                                             | 180                                  | 266       |
| NH <sub>3</sub>                             | 14.8                                 | 33.3      |
| H <sub>2</sub> S                            | 12.5                                 | 28.1      |
| Sulfur                                      | 6.0                                  | 0.85      |
| Water                                       | Remainder                            | Remainder |
| NaCl, %w <sup>b</sup>                       | Corrosion Rate, mils/yr <sup>a</sup> |           |
|                                             | 0                                    | 2         |
| 0.25                                        | 2                                    | —         |
| 0.50                                        | 2                                    | 6         |
| 0.75                                        | 2                                    | 9         |
| 1.0                                         | 2                                    | —         |
| 2.5                                         | 2                                    | 7         |
| 5.0                                         | 2                                    | —         |

<sup>a</sup>From weight loss and exposure time. No localized attack observed.

<sup>b</sup>Basis total solution.

Table 1 indicates the corrosion rate of carbon steel at 266°F in a high strength (33%w NH<sub>3</sub>, 28%w H<sub>2</sub>S) ammonium sulfide solution containing various amounts of sulfur present as polysulfide ions. A polysulfide solution containing 0.25%w sulfur was apparently on the borderline for inhibiting corrosion at 266°F as evidenced by the wide range in corrosion rate observed (6 to 270 mils/yr). With more sulfur present (>0.5%w),

the corrosion rate in the liquid was less than 10 mils/yr at this temperature. In general, higher strength solutions and higher temperatures require more sulfur present as polysulfide for inhibition of corrosion of carbon steel. When adequate sulfur was present (0.5%w) in the ammonium sulfide, the presence of salt (up to 2.5%w as NaCl) had no effect on its corrosivity to carbon steel (see Table 2).

An advantage of the present process for transporting through pipelines sulfur-liquid hydrocarbon slurries is that the slurry can be also prepared by direct injection of molten sulfur into a suitable liquid hydrocarbon as described in U.S. Pat. No. 2,798,772, and the ammonium polysulfide or ammonium hydrosulfide can be added in the slurry preparation vessel so that a non-corrosive slurry can be injected into the pipeline without additional requirement of ammonium polysulfide or ammonium hydrosulfide injection into the pipeline transporting the slurry. Other processes known to the art can be used to make the sulfur-liquid hydrocarbon slurry depending on the availability of the liquid carriers and slurry preparation conditions.

At the terminal end of the line the water phase can be readily removed by phase separation, and the sulfur can be removed from the liquid hydrocarbon by suitable means such as described in U.S. Pat. No. 2,798,772. The sulfur can be purified by methods as described in U.S. Pat. Nos. 2,809,885 or 3,489,677 which involves treating oil contaminated sulfur with an

aqueous solution containing a mixture of alkali hydrosulfide and corresponding hydroxide, e.g., ammonium hydrosulfide and ammonium hydroxide, or by other suitable means such as recovery of the sulfur from the oil slurry by filtration of molten sulfur and liquid-liquid extraction with a hydrocarbon solvent containing 10 to 50% by weight aromatics. At the receiving terminal the sulfur slurry can be filtered and washed. The recovered sulfur is then melted and purified by liquid-liquid extraction with an aromatic hydrocarbon such as cumene. Also, if desired, the filtered sulfur can be steam stripped to recover bright yellow sulfur.

I claim as my invention:

1. A method for preventing the sulfur corrosion of ferrous materials in contact with a sulfur-hydrocarbon slurry comprising admixing ammonium polysulfide with the slurry, the ammonium polysulfide comprising an aqueous solution of from about 0.01% to about 10% by weight based on total slurry.
2. A method for preventing the sulfur corrosion of ferrous materials in contact with a sulfur-hydrocarbon slurry comprising admixing ammonium polysulfide with the slurry, the ammonium polysulfide being formed at least in part by reacting ammonium hydroxide with free sulfur in the slurry, the ammonium hydrosulfide comprising an aqueous solution of from about 0.01% to about 10% by weight based on total slurry.

\* \* \* \* \*

30

35

40

45

50

55

60

65